

## [54] METHOD FOR PRODUCING EFFICIENTLY A HIGH TOUGHNESS AND HIGH TENSILE STRENGTH STEEL MATERIALS

[75] Inventors: **Hiroshi Sekine; Tadakatsu Maruyama**, both of Tokyo; **Katsutoshi Yamada**, Tokai, all of Japan[73] Assignee: **Nippon Steel Corporation**, Tokyo, Japan[22] Filed: **Oct. 15, 1973**[21] Appl. No.: **406,283**

## [30] Foreign Application Priority Data

Oct. 19, 1972 Japan ..... 47-103991

[52] U.S. Cl. .... 148/12 F

[51] Int. Cl. .... C21D 7/14

[58] Field of Search ..... 148/12 F

## [56]

## References Cited

## UNITED STATES PATENTS

|           |        |                     |          |
|-----------|--------|---------------------|----------|
| 3,328,211 | 6/1967 | Nakamura .....      | 148/12 F |
| 3,645,801 | 2/1972 | Melloy et al. ....  | 148/12 F |
| 3,726,723 | 4/1973 | Coldren et al. .... | 148/12 F |

Primary Examiner—W. Stallard

Attorney, Agent, or Firm—Toren, McGeady and Stanger

## [57] ABSTRACT

A method for producing efficiently a high toughness and high tensile strength steel material which comprises heating a low-carbon or low-carbon low-alloy steel slab and hot rolling the slab, said hot rolling step comprising giving the slab at least one reduction with reduction amount and temperature to be determined by  $N\sqrt{R_o/H}$  in which  $R_o$  is the roll radius(mm) of the rolling mill,  $N$  is the roll rotation (rpm) and  $H$  is the slab thickness before the reduction.

10 Claims, 3 Drawing Figures



FIG. 1



FIG. 2



FIG. 3



**METHOD FOR PRODUCING EFFICIENTLY A HIGH TOUGHNESS AND HIGH TENSILE STRENGTH STEEL MATERIALS**

The present invention relates to a method for producing steel materials through hot rolling including steel materials which have a thickness of more than 6mm and are used as rolled, and more particularly relates to efficient production of high toughness and high tensile strength steel materials or their intermediate products using Si-Mn steel or Nb-containing steel materials under specific rolling conditions.

In case of Nb-containing steels, it has been conventionally possible to obtain high strength easily, but various proposals have been made for restricting the rolling conditions in order to assure high toughness. For example, according to a Japanese patent publication Sho 40-28241 the slab heating temperature is restricted to a temperature not higher than 1190°C, and the final reduction is conducted at a temperature not higher than 1000°C. According to a Japanese patent publication Sho 44-27139, the slab is heated to a temperature not lower than 1230°C and then given a total reduction of more than 50% of the initial thickness of the slab at a temperature not lower than 1100°C, and in the successive rolling, the steel is further given in a temperature range of 850° to 700°C a total reduction of not less than 30% of the plate thickness at 850°C to finish the rolling. Further according to Japanese patent publication Sho 47-506, the total reduction at a temperature not higher than 1015°C is increased and the finishing rolling is conducted in a temperature range of 900° to 780°C and each of the last five reductions is restricted to 5% or more.

The above conventional rolling methods have defects that production efficiency is remarkably lowered and considerable product rejects are caused due to shape defects, because the slab heating temperature must be lowered than ordinarily, or the reduction amount in the low temperature range must be increased, or the rolling must be continued down to low temperatures. Particularly, in order to assure the total reduction amount or the finish of the rolling in the low temperature zone, it is necessary to stop the rolling operation to wait for the temperature lowering of the slab. It is a very important problem to decide the temperature range, or the plate thickness at which the rolling is stopped, but this is very difficult and complicated because it depends on mill designs, slab thickness and product thickness in each of rolling shops as reported in "Iron and Steel Institute Special Report", page 104, Vol. 110/122. This means that success in one mill shop or in one product can not be assured for other shops or products, and actually a plant experiment of considerably large scale has been required for each of the shop or product.

The present invention has established a hot rolling method which can solve the above defects or remarkably alleviate them and which can produce not only high tensile strength steels which can be used as rolled but also any high tensile strength steel obtained through rolling operation.

The features of the present invention are:

A. A method for producing efficiently a high toughness and high tensile strength steel which comprises subjecting a low-carbon steel slab or a low-carbon low alloy steel slab to hot rolling comprising heating the slab and giving the slab at least one reduction at a defi-

nite reduction temperature and reduction corresponding to  $N \sqrt{R_o/H}$  in which  $R_o$  is the radius of the rolling mill,  $N$  is the rotating speed (rpm) of the roll and  $H$  is the slab thickness (mm) before the reduction.

5 B. A method for producing efficiently a high toughness and high tensile strength steel which comprises hot rolling a low-carbon steel slab or a low-carbon low alloy steel slab, in which hot rolling the first reduction is started at a temperature of 1150°C and lower and at least one reduction under the condition defined by  $N \sqrt{R_o/H}$  as in (A) above is given to the slab.

10 According to the present invention, the following steps are preferably added in single or in combination to the above steps;

15 1. In the case of Nb-containing steel materials, the rolling is done in such a manner that the total reduction from 950°C and below to the finish of the rolling is not less than 45% of the slab thickness at 950°C, and the rolling is finished in a temperature range from 880°C to 20  $A_{r3}$  point of the steel material.

25 2. In case of Si-Mn steel materials, the rolling is effected so that the total reduction from 820°C to the rolling completion is not less than 20% of the slab thickness at 820°C, and the rolling is finished at a temperature range from 800°C to the  $A_{r3}$  point of the steel material.

30 3. In (1) or (2), rapid cooling is conducted after the finish of the rolling with an average cooling rate between 8°C/sec. and 40°C/sec. and the strip is coiled at a temperature between 680° and 550°C.

35 Reasons for limitations of the rolling conditions and the steel compositions in the present invention will be explained in detail hereinunder.

40 It is known that an appropriate addition of Nb in a low carbon steel will retard recrystallization of austenite after the hot rolling, and in case of Nb-containing steel which have been rolled fully at a low temperature, the transformation from the non-recrystallized austenite elongated in the rolling direction to ferrite is caused, and the nuclei of the ferrite grains generating at the time of the transformation are considerably greater in their number than when the isotropic austenite grains transform into the ferrite, so that the ferrite grains in 45 the Nb-containing steels which have been rolled at the low temperature are finer and the strength and toughness of the steel are improved, and it is also known that the above phenomenon appears in Si-Mn steels containing no niobium when the rolling temperature is low-

50 ered.

55 The present inventors have conducted extensive studies on the metallurgical processes during the hot rolling of the Nb-containing steels and Si-Mn steels and during the subsequent cooling thereof and have found that although it is very important for improvement of toughness of the Nb-containing steels and Si-Mn steels to finely recrystallize the austenite beforehand by the high temperature rolling, as disclosed in Japanese patent publication Sho 44-27139, this process can proceed at a temperature about 200°C lower than the lower limit temperature disclosed in the above prior art under certain conditions in case of Nb-containing steels for example, and it has been found that the basic condition of the rolling for refining the recrystallized austenite grains is not the total reduction down to the above lower limit temperature disclosed in the prior art, but it is to maintain each reduction higher than a certain definite value determined by various factors.

60 65

It has been further discovered that the recrystallization of, even during the reduction, is suddenly completed when a large reduction larger than another critical reduction which and is generally higher than the above limit reduction. In other words, this type of recrystallization should be called as a dynamic recrystallization and the dynamically recrystallized austenite grain size is directly determined as the function only of the reduction temperature and the average strain rate during the reduction.

It has been also found that the various factors which restrict the recrystallization behavior include the strain rate of the reduction which has never been considered in the conventional rolling art, in addition to the above reduction temperature and the grain size of austenite before the reduction.

If the recrystallization is called as static recrystallization in case when the recrystallization of austenite is completed a certain time after the reduction, the austenite grain size obtained by the dynamic recrystallization is always finer than that obtained by the static recrystallization when reduced under the same combination of the reduction temperature and the strain rate. This has been also discovered by the present inventors.

In a rolling process, it is known that the mean strain rate of a reduction,  $\dot{E}$ , is given by the following equation:

$$\dot{E} = \frac{2\pi}{60\sqrt{v}} N \sqrt{R_o/H} - \ln \frac{1}{1-r}$$

wherein  $r$  is the amount of reduction. The strain rate, which plays an important role in controlling the recrystallization behavior of the austenite is well defined only by the parameter  $N \sqrt{R_o/H}$ .

The reason for the limitation of the lower limit of each reduction in the rolling within the specific temperature zone in the present invention is that the present invention aims to positively refine the austenite grains through the dynamic recrystallization or at least through a rapid static recrystallization by each reduction in the above specific temperature range according to the above discovery.

The limitation of the temperature range of 1150° to 980°C for Nb-containing steels and 1150° to 850°C for Si-Mn steels in which the specific reduction is conducted is based on the discovery that the dynamic recrystallization is caused relatively easily even by the reduction schedule hitherto practised in rolling mills if the temperature is higher than 1150°C and a certain refinement of the austenite is attained, and that in case of the Nb-containing steels to which the present invention is applied, the dynamic recrystallization can proceed even by the reduction at 980°C at least if certain condition is satisfied, and similarly by the reduction at 850°C in case of Si-Mn steels.

The reason for defining the case in which the reduction is completely eliminated at temperatures above 1150°C is that in the case when high efficiency as a whole including steps prior to the hot rolling is obtained if the hot rolling is done with a relatively thin steel slab or in case when the product thickness is large, or in case when it is necessary to maintain the total reduction at the low temperature zone as defined in the additional feature (1) or (2) of the present invention for obtaining very high toughness, it is necessary to re-

duce the total reduction number in order to maintain each reduction between 1150° and 980°C or 1150°C and 850°C not smaller than the lower limit, and in such a case it is desirable for assuring the toughness to eliminate completely the reduction above 1150°C.

FIG. 1 and FIG. 3 show the results of extensive rolling experiments seeking for the lower limit reduction for the dynamic recrystallization of the austenite by each reduction between 1150°C and 980°C or between 10 1150°C and 850°C in relation to the reduction temperature, the rotating speed of the roll, the roll diameter and the plate thickness before the reduction, and these experiments were conducted on assumption of an ordinary process in which the Nb-containing steel or the 15 Si-Mn steel is given continuous reductions and, the austenite grains are gradually refined.

FIG. 2 shows results of experiments for determining the lower limit reduction necessary for the dynamic recrystallization of austenite grains to be caused when the 20 first reduction in the temperature range between 1150° and 1050°C is given to the Nb-containing steel which has been heated at high temperatures as usually and particularly about 1200°C at which the austenite grains 25 remarkably coarsen and cooled without any reduction down to 1150°C at all. The lower limit reduction is shown as the function of the various rolling conditions as in FIG. 1. Reasons for the definition that at least one reduction larger than those defined in FIG. 1 and FIG. 2 is given are that when only one reduction most disadvantageous to the refinement of the austenite is given under the condition using a strong rolling mill, recrystallized grains of more than No. 5 of the austenite grain 30 size are obtained and if the production process is conducted thereafter in combination with the desirable steps of (1), (2) and (3) a satisfactory fine structure of transformation product can be obtained and satisfactorily high strength and toughness are assured for the final products.

40 In the present invention, Nb-containing steels and Si-Mn steels are described separately because the presence of Nb changes considerably the lower limit reduction for the dynamic recrystallization and the reason for the limitation of the carbon content to 0.30% or less 45 in the steel composition applicable to the present invention is that more than 0.30% carbon remarkably deteriorates weldability of the steel and thus undesirable for the steel which requires rolling operations. Reason for the limitation of the niobium content to 0.15% or less in the steel composition in Nb-containing steels is that if the niobium content is more than 0.15%, it is impossible to prevent the raising the lower limit of the 50 temperature at which the austenite can be recrystallized during the rolling, and thus the conditions defined in FIG. 1 are changed even when the carbon and niobium contents are considerably reduced. Further, the alloying elements other than carbon and niobium are not specifically limited in the present invention because it has been confirmed through experiments that the 55 above facts are not changed quantitatively when Si, Mn, Ni, Cr, Cu and V are varied substantially.

In case of Si-Mn steels containing no niobium, silicon and manganese are dispensable for increasing the strength at low cost, but silicon contents more than 60 0.70% coarsen the ferrite grains, and manganese contents more than 2.0% cause problems in the steel making process and in connection with weldability. Thus the upper limits of these elements are defined as above.

Further, not only the steel materials which are used as rolled and steel materials of ferrite-pearlite structure, but also any high-tensile steel material to be obtained through hot rolling is included in the scope of the present invention. This is based on the following known facts and newly discovered facts. In case when the structure after cooling is mainly of bainite, even when the steel is quenched immediately after or a certain time after the rolling and then tempered, the finer the austenite before the transformation is, the better the toughness of the product is. Also in case when the steel is left to cool or is cooled at controlled cooling rate after the rolling, reheated, quenched and tempered or normalized, the finer the structure after the hot rolling and the cooling is, the more improved the toughness of the product is.

The present invention is based on the completely new discoveries including the results of the quantitative experiments and has been established as a controlled rolling method in which the rolling pass schedule in the high temperature range is controlled, and at least one large reduction is given in the high temperature range. This is completely different from the conventional controlled rolling method in which the rolling pass schedule in the low temperature is controlled.

As the result, according to the present invention, if the design is made in such a manner that the austenite recrystallization by the rolling at the specific high temperature range is occupied mainly by the dynamic recrystallization, the considerations to the temperature and the time as disclosed in the "Iron and Steel Institute Special Report" for waiting for the slab temperature lowering by stopping the rolling operation in the specific temperature range are not required.

Further according to the present invention, the rolling at the high temperatures where the steel material is still soft enough is controlled so as to refine the austenite and to assure the same level of toughness, while the rolling at low temperature where the steel material becomes hard is alleviated, the waiting time for the slab temperature lowering for the low temperature is saved, thus increasing the production efficiency, reducing the defects such as plate waviness and crowns due to the low temperature rolling, improving the production yield, and making possible to effect the rolling by a relatively light rolling mill.

Further the present invention has advantages that only by incorporating the effects of strain rate into the rolling schedule it is no more necessary to translate with great efforts a successful rolling operation at a specific rolling shop or with a specific plate thickness into a rolling operation of different specification, and it is possible to produce good rolled products only with a minimum plant experiments at a rolling shop having no experience of controlled rolling. The above advantages of the present invention have great industrial significance.

As above mentioned, it is one of the features of the present invention to select the rolling conditions so as to make the austenite take the dynamic recrystallization between 1150° and 980°C or 1150° and 850°C, but it should be understood that the present invention also include the cases in which the recrystallization of the austenite in the above temperature range is not the dynamic recrystallization, that is, the recrystallization is completed a certain time after the reduction.

The reasons are as follows: the curves in FIGS. 1 and 3, or the curves in FIG. 2 have been respectively sought

for on the basis of the austenite grain size when the ordinary reduction schedule is given or the austenite grain size before the first reduction when the average slab heating is effected. Therefore, it is probable that

5 the dynamic recrystallization does not take place but instead the static recrystallization takes place depending on the slab heating or the rolling history up to the reduction specified by the present invention even when the rolling conditions of FIGS. 1 to 3 are satisfied. Even

10 in this case, if each of the reductions is made so large, the completion of the recrystallization is promoted and the recrystallized grains are refined, and thus most of the objects of the present invention can be attained.

In the present invention, the following alloying elements may be added in addition to C, Mn, and Nb for various purposes in combination with the additional production conditions of (1) to (3).

According to the present invention, the reductions in the high temperature range of 1150° to 980°C or 1150° to 850°C are specified, but when the low temperature rollings as specified in (1) and (2) are applied in combination, the strength and toughness can be further improved.

The above technical thought has some connection with the rolling type in which the rolling pass schedule in the low temperature range is controlled, but the temperature of 950°C or lower for Nb-containing steel or of 820°C or lower for Si-Mn steel defined for the total reduction and the temperature of 880°C or lower for

25 Nb-containing steel or of 800°C or lower for Si-Mn steel defined for the hot rolling completion are high as compared with the conventional arts. Namely, in the present invention, the restrictions in the low temperature range are alleviated as compared with the conventional art for the production of the same steel grades by specifying the high temperature rolling conditions, thus improving the production efficiency and yield.

The cooling and the coiling conditions after the rolling as defined in the preferably condition (3) are directed to the case when the structure after the coiling is mainly of ferrite-pearlite. It is known that the intermingling of the bainite into the structure after the transformation is harmful for the toughness of the steel material, and it has been found that it is effective for the refinement of the ferrite to effect a rapid cooling at the time of the transformation so far as the bainite is not present.

In a continuous rolling, when the cooling after the rolling is made rapid and the coiling temperature is lowered, the ferrite becomes finer, but the bainite appears during the cooling or after the coiling under a certain condition. This limit cooling rate is 40°C/sec. and the limit cooling temperature is 550°C.

The cooling rate of 8°C/sec. corresponds to the considerable slow cooling side of the conventional continuous hot rolling, and at such a cooling rate the coiling will be naturally a high temperature coiling. The low temperature coiling enhances the effectiveness of precipitation hardening by Nb, and V. Therefore, with a cooling rate as slow as 8°C/sec. the strength is naturally low but excellent toughness is assured.

It is preferable to add 0.01 to 0.70% Si and 0.70 to 2.00% Mn to the Nb-containing steel too, from the necessity of the steel making and for assuring the strength at low cost. Lowering of the carbon is also preferable for assuring the toughness and the weldability, but in case of ferrite-pearlite steels in particular, the increase of the transformation temperature thereby is not desir-

able because it reduces the precipitation hardening by Nb, and V, coarsens the ferrite grains and deteriorates the toughness. Therefore, in the case of Nb-containing steels it is preferable to define (C + Mn + Nb)  $\geq 1.35\%$ .

Niobium, when added with the other elements, is effective to improve the toughness and strength, but should be maintained lower from the point of weldability. It also changes partially the conditions shown in FIG. 1 through its precipitation of NbN into the austenite. Therefore it is preferable to maintain the nitrogen content not more than 0.010%.

Further, not more than 0.08% Al may be added from the necessity of the steel making, not more than 0.20% V may be added for obtaining desirable strength, not more than 0.005% B may be added for assuring hardenability as required for tempered steels, not more than 1.50% Ni may be added for assuring the toughness, strength and the transformation temperature, not more than 2.00% Cu may be added for the corrosion resistance and the strength, not more than 1.00% Cr may be added for the strength and the transformation temperature, not more than 0.20% Ce or misch metal may be added for controlling the shape of sulfides and improving the toughness and workability in the direction perpendicular to the rolling direction, and not more than (0.15 - Nb%) Ti only for Nb-containing steel or not more than 0.10% Zr may be added for adjusting the shape of sulfides, absorbing N, and restricting the coarsening of the austenite grains during the reheating. The above additions do not substantially change the limit reduction defined in FIGS. 1 and 3. The reason for limiting the titanium content in connection with the ni-

The Nb-containing killed steels A and B which were prepared in a converter were made into flat slabs of 240mm thickness, heated 1300°C, rolled to 82mm thickness by three reductions down to 1150°C, subjected to the reduction at three temperatures in combination as shown in Table 3 at a constant reduction as shown in Table 2 using the roll groups specified in Table 2 for the fourth, fifth and sixth reductions, and then further rolled into 9mm thickness by twelve reductions in total, and coiled at 650°C. The rolling schedule 1 in Table 3 represents an ordinary rolling with no restriction, and the rolling schedules 2 and 3 in which the temperature was restricted had longer rolling times than the ordinary rolling schedule 1 by 50 and 90 seconds respectively. Table 3 shows also the values of  $N \sqrt{R_o/H}$  and the lower limit reduction values determined from FIG. 1 for the dynamic recrystallization sought for from the reduction temperatures shown in Table 3.

20

Table 2

|    |                                        | Specification of Rolling Mill and Reduction Allotment |                 |                 |
|----|----------------------------------------|-------------------------------------------------------|-----------------|-----------------|
|    |                                        | Fourth Reduction                                      | Fifth Reduction | Sixth Reduction |
| 25 | Roll Radius<br>(mm)                    | 457                                                   | 457             | 365             |
|    | Rotating Speed of Roll<br>(rpm)        | 46.8                                                  | 59.3            | 42.7            |
| 30 | Change in Slab<br>Thickness<br>(mm/mm) | 82/48                                                 | 48/31           | 31/24.5         |
|    | Reduction (%)                          | 41.3                                                  | 35.1            | 21.0            |
|    | $N \sqrt{R_o/H}$ (rpm)                 | 110                                                   | 183             | 147             |

Table 3: Rolling Temperatures and Lower Limit Reductions for Dynamic Recrystallization

| Rolling Schedule | Fourth Reduction | Fifth Reduction  |                           | Sixth Reduction  |                           | Final Reduction Temperature (°C) |
|------------------|------------------|------------------|---------------------------|------------------|---------------------------|----------------------------------|
|                  |                  | Temperature (°C) | Lower Limit Reduction (%) | Temperature (°C) | Lower Limit Reduction (%) |                                  |
| 1                | 1100             | 27.5             | 1070                      | 31.0             | 1000                      | 38.5                             |
| 2                | 1100             | 27.5             | 1030                      | 34.5             | 960                       | —                                |
| 3                | 1100             | 27.5             | 1030                      | 34.5             | 930                       | —                                |
|                  |                  |                  |                           |                  |                           | 830                              |

obium content is that the titanium addition also contributes to restrict the austenite recrystallization during the hot rolling similarly as the niobium content.

The present invention will be more clear from the following examples.

#### EXAMPLE 1

Table 1 shows the chemical compositions of the steel materials used in present invention.

Table 1

| Chemical Compositions of Steel Materials (in weight %) |      |      |       |       |      |      |
|--------------------------------------------------------|------|------|-------|-------|------|------|
| C                                                      | Si   | Mn   | P     | S     | Nb   | V    |
| A 0.11                                                 | 0.24 | 1.01 | 0.017 | 0.010 | 0.03 | —    |
| B 0.11                                                 | 0.25 | 1.30 | 0.020 | 0.007 | 0.03 | —    |
| C 0.10                                                 | 0.25 | 1.26 | 0.010 | 0.005 | 0.03 | 0.05 |

55 From the comparison of Tables 2 and 3, the followingings are clear. In Table 3, the rolling schedule 1 satisfies the present invention in its fourth and fifth reductions, but includes the sixth reduction between 1150° and 980°C which does not satisfy the present invention and thus is outside the scope of the present invention. Whereas in the rolling schedules 2 and 3, not only the fourth and fifth reductions satisfy the present invention, but also the sixth reduction is effected at temperatures not higher than 980°C and thus no restriction for the reduction is required. Namely the rolling schedules 2 and 3 are within the scope of the present invention. Mechanical properties at the coil center portion of the steel strip thus obtained are shown in Table 4.

Table 4

| Sample Steels | Rolling Schedule | Mechanical Properties of Rolled Steels (A and B) |                                        |                |                                           |                            |                                |
|---------------|------------------|--------------------------------------------------|----------------------------------------|----------------|-------------------------------------------|----------------------------|--------------------------------|
|               |                  | Yield Point (Kg/mm <sup>2</sup> )                | Tensile Strength (Kg/mm <sup>2</sup> ) | Elongation (%) | vE <sub>-40</sub> <sup>(T)</sup> = (Kg-m) | vTrs <sup>(T)</sup> = (°C) | dwtt Trs <sup>(T)</sup> = (°C) |
| A             | 1                | 37/40                                            | 49/49                                  | 39/31          | 1.2/2.8                                   | -30/-50                    | -21/-42                        |
|               | 2                | 38/42                                            | 50/52                                  | 38/32          | 2.5/2.9                                   | -52/-68                    | -41/-54                        |
|               | 3                | 43/47                                            | 54/56                                  | 36/29          | 1.7/2.6                                   | -44/-74                    | -23/-42                        |
| B             | 1                | 37/40                                            | 51/52                                  | 38/32          | 3.2/3.6                                   | -52/-74                    | -43/-48                        |
|               | 2                | 40/45                                            | 54/56                                  | 38/29          | 2.7/3.0                                   | -67/-74                    | -53/-62                        |
|               | 3                | 42/46                                            | 55/57                                  | 37/28          | 2.6/3.0                                   | -63/-78                    | -49/-55                        |

\*2% sub-size

Tensile Properties: Rolling Direction/Perpendicular to Rolling Direction

Toughness: Worst/Best

It is understood from the comparison of the rolling conditions shown in Table 3 and the mechanical properties shown in Table 4 that both of the strength and the toughness of the steels A and B obtained by the rolling schedules 2 and 3 are better than those obtained by the rolling schedule 1. It is also understood from the comparison of the schedules 2 and 3 that the schedule 3 in which the waiting time of 40 seconds in the course of the rolling for assuring the low temperature rolling shows somewhat higher strength for both of the steels A and B than the schedule 2, but shows no tangible improvement in the toughness. Whereas the schedule 2 gives very stable toughness as compared with the schedules 1 and 3. The schedule 2 is the typical embodiment of the present invention which can produce a high toughness and high tensile strength steel at a high production efficiency without applying a very low temperature rolling.

#### EXAMPLE 2

The killed steel C containing Nb and V, prepared in a convertor and having the chemical composition shown in Table 1 was made into a flat slab of 215mm thickness, heated to 1300°C, and rolled to 76mm thickness by three reductions down to 1150°C, subjected to three rolling schedules with the combination of the reduction temperatures and the reductions shown in Table 5, using the roll groups shown in Table 2 for the fourth, fifth and sixth reductions, further rolled to 12.7mm thickness by eleven reductions in total, and coiled at the temperatures shown in Table 5.

The rolling schedule 4 in Table 5 represents an ordinary rolling with no restriction. The schedule 5 had a longer rolling time than the ordinary rolling schedule by 60 seconds, and in the rolling schedule 6, waiting

time was of 70 seconds provided on the waiting side table between the fourth and the fifth reductions.

The figures in the parenthesis in Table 5 represent the lower limit reduction amount for the dynamic recrystallization for each reduction sought for from FIG. 1 on the basis of the value of  $N \sqrt{R_o/H}$  and the reduction temperatures in the table. The rolling schedule 4 in Table 5 includes the sixth reduction which does not reach the lower limit reduction amount determined from FIG. 1 between 1150° and 980°C, while in the rolling schedules 5 and 6, the fourth and the fifth reductions are over the reduction amounts given by FIG. 1 and yet the sixth reduction is 970°C in the schedule 5 and 965°C in the schedule 6, both being outside the restricted temperature range. Thus the schedules 5 and 6 are within the scope of the present invention.

The mechanical properties of the steel strips thus rolled are shown in Table 6, from which it is clear that the schedules 5 and 6 give excellent strength and toughness in spite of the thickness of 12.7mm as compared with the schedule 4. Remarkable amount of bainite was observed in some of the steel materials rolled by the schedule 4 in spite of the high temperature coiling, while in the steel materials rolled by the schedules 5 and 6, no such structure was observed. The extension of rolling time of 60 seconds in the schedule 5 causes only about 30% lowering in the production efficiency in the continuous hot rolling mill where the present invention was applied. In schedule 6, the lowering of the production efficiency was completely eliminated by the use of the side table. Thus it is understood that the present invention represented by the schedules 5 and 6 assures remarkable efficiency for the production of steel plates of thickness and quality as above.

Table 5

|                                   | Rolling Schedules and Lower Limit Reductions for Dynamic Recrystallization |                 |                 |       | Temperature of Final Reduction | Cooling Temperature |  |  |
|-----------------------------------|----------------------------------------------------------------------------|-----------------|-----------------|-------|--------------------------------|---------------------|--|--|
|                                   | Fourth Reduction                                                           | Fifth Reduction | Sixth Reduction |       |                                |                     |  |  |
|                                   |                                                                            |                 |                 |       |                                |                     |  |  |
| Changes in Slab Thickness (mm/mm) | 76/46                                                                      | 46/31           | 31/24.5         |       | —                              | —                   |  |  |
| Reduction (%)                     | 39.5                                                                       | 32.6            | 21.0            |       | —                              | —                   |  |  |
| $N \sqrt{R_o/H}$ (rpm)            | 115                                                                        | 187             | 147             |       | —                              | —                   |  |  |
| Schedule 4                        | 1120°C(26.0%)                                                              | 1110°C(30.1%)   | 1030°C(32.0%)   | 880°C | 715°C                          |                     |  |  |
| Schedule 5                        | 1140°C(23.0%)                                                              | 1050°C(32.0%)   | 970°C(—)        | 873°C | 695°C                          |                     |  |  |
| Schedule 6                        | 1130°C(25.0%)                                                              | 1030°C(32.5%)   | 965°C(—)        | 867°C | 680°C                          |                     |  |  |

Table 6

| Rolling Schedule | Yield Point (Kg/mm <sup>2</sup> ) | Tensile Strength (Kg/mm <sup>2</sup> ) | Mechanical Properties of Rolled Steel (C) |                                         |                          |         | dwtt Trs <sup>(T)</sup> (°C) | Sample-Taking Position (From the rolling head) |
|------------------|-----------------------------------|----------------------------------------|-------------------------------------------|-----------------------------------------|--------------------------|---------|------------------------------|------------------------------------------------|
|                  |                                   |                                        | Elongation (%)                            | vE <sub>-40</sub> <sup>(T)</sup> (Kg-m) | vTrs <sup>(T)</sup> (°C) |         |                              |                                                |
| 4                | 38/43                             | 55/56                                  | 38/37                                     | 0.9/1.5                                 | —                        | +20     | 75%                          |                                                |
| 5                | 34/37                             | 50/52                                  | 42/37                                     | 1.8/5.4                                 | -33/-53                  | -25/-43 | 21%                          |                                                |
| 6                | 40/44                             | 56/58                                  | 38/36                                     | 2.2/4.5                                 | -28/-45                  | -23/-34 | 32%                          |                                                |
| 7                | 37/39                             | 54/55                                  | 40/35                                     | 3.0/5.8                                 | -31/-52                  | -25/-30 | 10%                          |                                                |

Tensile Properties: Rolling Direction/Perpendicular to Rolling Direction:  
Toughness: Worst/Best

## EXAMPLE 3

Steel C containing niobium and vanadium shown in Table 1 made into flat slabs of 100mm thickness, heated to 1250°C, cooled without any reduction down to 1150°C and three reductions were made between 1150° and 980°C according to the rolling schedule shown in Table 7, using the roll groups shown in Table 7 for the first and the third reductions, and subsequent rolling was made to obtain steel plates of 12.9mm thickness with the total nine reductions and the plates were coiled at 670°C. The figures in the parenthesis in Table 7 the lower limit reduction amounts for the dynamic recrystallization for each reduction, determined from FIG. 2 for the second reduction, from FIG. 1 for the first and third reductions on the basis of the values of  $N \sqrt{R_o/H}$  and the reduction temperatures. From Table 7 it is understood that the rolling schedule 7 satisfies the rolling conditions of the present invention.

Table 7

|                                   | Specification of Rolling Mill, Rolling Schedule and Lower Limit Reductions for Dynamic Recrystallization |                  |                 |                 |
|-----------------------------------|----------------------------------------------------------------------------------------------------------|------------------|-----------------|-----------------|
|                                   | First Reduction                                                                                          | Second Reduction | Third Reduction | Final Reduction |
| Roll Radius (mm)                  | 559                                                                                                      | 457              | 457             | —               |
| Rotating Speed of Roll (rpm)      | 28.7                                                                                                     | 46.8             | 59.3            | —               |
| Changes in Slab Thickness (mm/mm) | 100/69                                                                                                   | 69/48            | 48/31           | —               |
| Reduction (%)                     | 31.0                                                                                                     | 30.4             | 35.4            | —               |
| $N \sqrt{R_o/H}$ (rpm)            | 60                                                                                                       | 115              | 187             | —               |
| Rolling Schedule                  | 1140°C                                                                                                   | 1110°C           | 1020°C          | 865°C           |
| 7                                 | (30.0%)                                                                                                  | (27.0%)          | (35.0%)         |                 |

The mechanical properties near the coil head portion of thus rolled steel plates are shown at the lowest column in Table 6. It is understood that the schedule 7 which is within the scope of the present invention gives better material properties than the schedule 5 in spite of the thickness of 12.9mm. This example represents a case where the thickness of slabs introduced to a rolling mill is relatively thin. Even in such a case, a fine structure which gives desired excellent strength and toughness can be obtained by completely eliminating reductions above 1150°C and by increasing enough the amount of the first reduction at temperatures lower than 1150°C. Almost no intermingling of bainite was observed in the rolled structure of the above material.

## EXAMPLE 4

The killed steel D shown in Table 8 containing Nb and V, which was prepared in a convertor was made into flat slabs of 220mm thickness, heated to 1250°C, and rolled according to the two rolling schedules shown

in Table 9, using the rpm-variable rolls of 500mm radius to obtain steel plates of 19mm thickness.

Table 8

| C    | Si   | Chemical Composition of Steel D |      |       |       |       |
|------|------|---------------------------------|------|-------|-------|-------|
|      |      | Mn                              | P    | S     | Nb    | V     |
| 0.11 | 0.27 | 1.41                            | 0.02 | 0.006 | 0.032 | 0.035 |

In the rolling schedule 8 in Table 9, the reductions of the fourth and fifth reductions are larger than the lower limit reduction amount for the dynamic recrystallization, and thereafter subsequent reductions were started at 880°C and total reduction of 70% was effected between 880°C and 780°C, and thus the schedule 8 is within the scope of the present invention. Whereas in the schedule 9, low reductions below the lower limit reduction amount for the dynamic recrystallization were conducted at temperatures not lower than 990°C, and

thus outside the scope of the present invention, but the lower temperature reductions were made at far lower temperatures and the total reduction in the low temperature zone is greater as compared with the schedule 8.

Mechanical testings were done on the top, middle and bottom portions of the steel plates rolled and the measurements as average of the three portions are shown in Table 10.

From the comparison of the mechanical properties shown in Table 10 and the rolling conditions shown in Table 9 it is understood that the schedule 8 which is within the scope of the present invention gives better strength and toughness than the schedule 9 which is outside the scope of the present invention. In case of the steel plates which were rolled by the schedule 8, despite the thickness of 19mm and the fact that the lower temperature zone reductions which remarkably lower production yield and efficiency were not strengthened particularly, excellent strength and toughness due to a uniform structure of very fine grains of ferrite grain

number of about 12.5 are obtained. This means that the present invention is useful for production of such thick steel plates.

amount for the dynamic recrystallization, and the subsequent reductions were started from 800°C, with the total reduction of 25% between 800° and 750°C. Thus

Table 9

| Schedule 8                   | Rolling Conditions and Lower Limit Reduction for Dynamic Recrystallization |                  |                 | Low Temperature Rolling Condition       |
|------------------------------|----------------------------------------------------------------------------|------------------|-----------------|-----------------------------------------|
|                              | Third Reduction                                                            | Fourth Reduction | Fifth Reduction |                                         |
| Rotating Speed of Roll (rpm) | 29                                                                         | 21               | 44              | 63 to 19mm thickness                    |
| Changes in Slab              | 166/133                                                                    | 133/97           | 97/63           | 7 passes (880/780°C)                    |
| Thickness (mm/mm)            |                                                                            |                  |                 | Finishing Temperature 780°C             |
| Reduction (%)                | 19.9                                                                       | 27.1             | 35.1            | Total Reduction in Low Temperature Zone |
| $N \sqrt{R_o/H}$ (rpm)       | 51                                                                         | 41               | 100             | 70%                                     |
| Reduction Temperature (°C)   | 1100                                                                       | 1080             | 1010°C          |                                         |
| Lower Limit Reduction (%)    | 24                                                                         | 23               | 33.5            |                                         |

  

| Schedule 9                   | Rolling Conditions and Lower Limit Reduction for Dynamic Recrystallization |                   |                  | Low Temperature Rolling Condition       |
|------------------------------|----------------------------------------------------------------------------|-------------------|------------------|-----------------------------------------|
|                              | Sixth Reduction                                                            | Seventh Reduction | Eighth Reduction |                                         |
| Rotating Speed of Roll (rpm) | 28                                                                         | 31                | 31               | 79 to 19mm thickness                    |
| Changes in Slab              | 121/105                                                                    | 105/91            | 91/79            | 8 passes 1830/730°C                     |
| Thickness (mm/mm)            |                                                                            |                   |                  | Finishing Temperature 730°C             |
| Reduction (%)                | 13.2                                                                       | 13.3              | 13.2             | Total Reduction in Low Temperature Zone |
| $N \sqrt{R_o/H}$ (rpm)       | 57                                                                         | 68                | 72               | 76%                                     |
| Reduction Temperature (°C)   | 1010                                                                       | 1000              | 990              |                                         |
| Lower Limit Reduction (%)    | 29                                                                         | 33                | 37               |                                         |

Table 10

| Rolling Schedule | Mechanical Properties of Steel D of 19mm Thickness |                           |                |                         |                   |                       |
|------------------|----------------------------------------------------|---------------------------|----------------|-------------------------|-------------------|-----------------------|
|                  | Yield Point (Kg/mm²)                               | Tensile Strength (Kg/mm²) | Elongation (%) | $vE_{-40}^{(T)}$ (Kg-m) | $vTrs^{(T)}$ (°C) | $dwtt Trs^{(T)}$ (°C) |
| 8                | 51/54                                              | 60/63                     | 42/37          | 5.4/6.8                 | -82/-90           | -50                   |
| 9                | 47/48                                              | 57/58                     | 44/46          | 6.4/8.0                 | -60/-70           | -40                   |

\* Measured at the middle portion of the steel plate.  
Tensile Properties: Rolling Direction/perpendicular to Rolling Direction: Toughness: Worst/Best

## EXAMPLE 5

The killed Si-Mn steel E prepared in a convertor and having the chemical composition shown in Table 11 was made into flat slabs of 245mm thickness, heated to 1250°C, and rolled according to the two rolling schedules shown in Table 12 using the rolls of 485mm radius of fixed rotation rate of 40 r.p.m. to obtain steel plates of 30mm thickness.

Table 11

| C    | Chemical Composition of Steel E |      |       |       |
|------|---------------------------------|------|-------|-------|
|      | Si                              | Mn   | P     | S     |
| 0.10 | 0.27                            | 1.36 | 0.013 | 0.005 |

Table 12 shows the values of  $N \sqrt{R_o/H}$ , the reduction temperature and the lower limit reduction amounts for the dynamic recrystallization for the Si-Mn steel determined from FIG. 3. In the schedule 10, the tenth reduction was over the lower limit reduction

40 the schedule 10 is within the scope of the present invention. Whereas in the schedule 11, low reductions below the lower limit reduction for the dynamic recrystallization were conducted at temperatures not lower than 1000°C and thereafter the reductions were made according to the same schedule 10. Thus the schedule 11 is outside the scope of the present invention.

45 Mechanical properties of the Si-Mn steel plates of 30mm thickness as rolled above are shown in Table 13 as average of the four portions from the top to the bottom.

50 When the mechanical properties shown in Table 13 and the rolling conditions shown in Table 12 are compared, it is understood that the schedule 10 which is within the scope of the present invention gives better strength and toughness than the schedule 11 which is outside the scope of the present invention. The results obtained by the schedule 10 clearly indicates that the present invention is useful for production of the Si-Mn steel plates as thick as of 30mm thickness and not containing alloying elements such as niobium.

Table 12.

| Finishing Rolling Ninth Reduction | Finishing Rolling Tenth Reduction | Low Temperature Rolling Condition |
|-----------------------------------|-----------------------------------|-----------------------------------|
|                                   |                                   |                                   |

Table 12.-continued

|                                         | Finishing<br>Rolling<br>Ninth<br>Reduction | Finishing<br>Rolling<br>Tenth<br>Reduction | Low Temperature<br>Rolling<br>Condition                    |
|-----------------------------------------|--------------------------------------------|--------------------------------------------|------------------------------------------------------------|
| (rpm)                                   |                                            |                                            | for schedules<br>9 and 10                                  |
| Changes in Slab<br>Thickness(mm/mm)     | 70/55                                      | 55/40                                      | 40 to 30mm<br>thickness<br>five reduction<br>(800°C-750°C) |
| Reduction (%)<br>$N \sqrt{R_o/H}$ (rpm) | 21.4<br>105                                | 27.3<br>119                                | Total Reduction<br>in low temper-<br>ature zone 25%        |
| Reduction Temper-<br>ature (°C)         | 1010                                       | 1000                                       |                                                            |
| Lower Limit                             |                                            |                                            |                                                            |
| Reduction (%)                           | 25                                         | 26                                         |                                                            |
| Schedule 11                             |                                            |                                            |                                                            |
| Rotating Speed of<br>Roll<br>(rpm)      | 40                                         | 40                                         |                                                            |
| Changes in Slab<br>Thickness(mm/mm)     | 65/50                                      | 50/40                                      |                                                            |
| Reduction (%)                           | 23.1                                       | 20.0                                       |                                                            |
| $N \sqrt{R_o/H}$ (rpm)                  | 109                                        | 125                                        |                                                            |
| Reduction Temper-<br>ature (°C)         | 1000                                       | 1000                                       |                                                            |
| Lower Limit                             |                                            |                                            |                                                            |
| Reduction (%)                           | 26                                         | 26.5                                       |                                                            |

Table 13

| Rolling<br>Schedule | Mechanical Properties of Steel E        |                                              |                        |                                  |                            |
|---------------------|-----------------------------------------|----------------------------------------------|------------------------|----------------------------------|----------------------------|
|                     | Yield<br>Point<br>(Kg/mm <sup>2</sup> ) | Tensile<br>Strength<br>(Kg/mm <sup>2</sup> ) | Elonga-<br>tion<br>(%) | $\sqrt{E_{-50}}^{(T)}$<br>(kg-m) | $\sqrt{Trs}^{(T)}$<br>(°C) |
| 10                  | 37/37                                   | 50/50                                        | 39/38                  | 2.0/7.0                          | -25/-44                    |
| 11                  | 31/32                                   | 48/49                                        | 39/38                  | 1.0/5.6                          | -13/-27                    |

Tensile Properties: Rolling Direction/Perpendicular to Rolling Direction Toughness: Worst/Best

What is claimed is:

1. A method for efficiently producing a high toughness and high tensile strength steel material which comprises heating a low-carbon or low-carbon, low-alloy steel slab which contains not more than 0.30% C, and not more than 0.15% Nb, and hot rolling the slab, said hot rolling step comprising giving the slab at least one reduction in an amount not smaller than that shown by each of the curves or the interpolated curves shown in FIG. 1 as determined by the constant  $N \sqrt{R_o/H}$  wherein  $R_o$  is the roll radius (mm) of the rolling mill, N is the roll rotation speed (rpm) and H is the slab thickness before the reduction.

2. A method for producing efficiently a high toughness and high tensile strength steel material, which comprises heating a steel slab containing not more than 0.30% C and not more than 0.15% Nb to a temperature required for assuring required strength of the steel slab, and hot rolling the slab, said hot rolling comprising giving the slab between 1150° and 980°C at least one reduction including a reduction conducted at the lowest temperature within the above temperature range with a reduction amount not smaller than that shown by each of the curves or the interpolated curves shown in FIG. 1 in accordance with the constant  $N \sqrt{R_o/H}$  as defined in claim 1 and the reduction temperature.

3. A method for producing efficiently a high toughness and high tensile strength steel material, which comprises heating a steel slab containing not more than 0.30% C, not more than 0.70% Si and not more than 2.00% Mn to a temperature required for assuring required strength of the steel slab, and hot rolling the

slab, said hot rolling comprising giving the slab between 1150° and 850°C at least one reduction including a reduction conducted at the lowest temperature within the above temperature range with a reduction amount not smaller than that shown by each of the curves or the interpolated curves shown in FIG. 3 in accordance with the constant  $N \sqrt{R_o/H}$  as defined in claim 1 and the reduction temperature.

4. A method according to claim 1 in which the first reduction is started at a temperature not higher than 1150°C.

5. A method according to claim 1 in which the first reduction is started at a temperature not higher than 1150°C.

6. A method for producing efficiently a high toughness and high tensile strength steel material, which comprises heating a steel slab containing not more than 0.30% C, and not more than 0.15% Nb to a temperature required for assuring required strength and hot rolling the steel slab, said hot rolling comprising starting the first reduction at a temperature not higher than 1150°C, giving the slab during the rolling between 1150° and 980°C including the first reduction at least one reduction including the reduction conducted at the lowest temperature within the above temperature range with a reduction amount not smaller than that shown by each of the curves or the interpolated curves shown in FIG. 1 in accordance with the constant  $N \sqrt{R_o/H}$  as defined in claim 1 and the reduction temperature.

7. A method for producing efficiently a high toughness and high tensile strength steel, which comprises

heating a steel slab containing not more than 0.30% C and not more than 0.15% Nb to a temperature not lower than 1200°C, hot rolling the slab, said hot rolling comprising starting the first reduction at a temperature not higher than 1150°C with a reduction amount not smaller than that shown by each of the curves or the interpolated curves shown in FIG. 2 in accordance with the constant  $N \sqrt{R_o/H}$  as defined in claim 1 and the reduction temperature, and conducting subsequent reductions down to 980°C including at least one reduction including the reduction at the lowest temperature between 1150 and 850°C with a reduction amount not smaller than that shown by each of the curves or the interpolated curves in FIG. 1.

8. A method for producing efficiently a high toughness and high tensile strength steel material, which comprises heating a steel slab containing not more than 0.30% C, not more than 0.70% Si, and not more than 2.00% Mn to a temperature required for assuring required strength and hot rolling the steel slab, said hot rolling comprising starting the first reduction at a temperature not higher than 1150°C, giving the slab during the rolling between 1150° and 850°C at least one re-

duction including the reduction conducted at the lowest temperature within the temperature range with a reduction amount not smaller than that shown by each of the curves or the interpolated curves in FIG. 3 in accordance with the constant  $N \sqrt{R_o/H}$  as defined in claim 1 and the reduction temperature.

9. A method for efficiently producing a high toughness and high tensile strength steel material which comprises heating a low-carbon or low-carbon, low-alloy steel slab which contains not more than 0.30% C, not more than 0.70% Si, and not more than 2.0 % Mn, and hot rolling the slab, said hot rolling step comprising giving the slab at least one reduction an an amount not smaller than that shown by each of the curves or the interpolated curves shown in FIG. 3 as determined by the constant  $N \sqrt{R_o/H}$  wherein  $R_o$  is the roll radius (mm) of the rolling mill, N is the roll rotation speed (rpm) and H is the slab thickness before the reduction.

10. A method according to claim 9 in which the first reduction is started at a temperature not higher than 1150°C.

\* \* \* \* \*

25

30

35

40

45

50

55

60

65

UNITED STATES PATENT OFFICE  
CERTIFICATE OF CORRECTION Page 1 of 3

Patent No. 3,918,999 Dated November 11, 1975

Inventor(s) Hiroshi Sekine; Tadakatsu Maruyama; Katsutoshi Yamada

It is certified that error appears in the above-identified patent and that said Letters Patent are hereby corrected as shown below:

Column 1, Line 36, change "conventional" to --prior--;  
Line 52, change "page 104, Vol. 110/122 to  
--Vol. 104, pages 110/122--;

Column 2, Line 37, change "rolling" to --reduction--;

Column 3, Line 26, change "G" to --E--;  
Line 31, the structural formula should appear  
as follows:

$$\dot{E} = \frac{2\pi}{60\sqrt{r}} N \sqrt{R_o/H} \cdot \ln \frac{1}{1-r}$$

Column 3, Line 36, after "N  $\sqrt{R_o/H}$ " insert --and r--;

Column 4, Line 23, change "about" to --above--;  
Line 28/29, change "and FIG. 2" to --or FIG. 3--;  
Line 52, after "raising" insert --of--;  
Line 55/56, change "niobium" to --nitrogen--;

Column 5, Line 62, change "shold" to --should--;  
Line 63, change "include" to --includes--;

Column 6, Line 3, change "average" to --conventional--;  
Line 15, after "C," insert --Si---;  
Line 21, change "rollings as specified in (1) and  
(2) are" to --rolling as specified in (1)  
or (2) is--;  
Line 33, change "conventional" to --prior--;  
Line 34/35, change "conventional" to --prior--;  
Line 46, after "transformation" insert --- and  
Line 46-47 delete "so far as the bainite is not  
present."

UNITED STATES PATENT OFFICE Page 2 of 3  
CERTIFICATE OF CORRECTION

Patent No. 3,918,999 Dated November 11, 1975

Inventor(s) Hiroshi Sekine; Tadakatsu Maruyama; Katsutoshi Yamada

It is certified that error appears in the above-identified patent and that said Letters Patent are hereby corrected as shown below:

Column 7, Line 6, change "Niobium" to --Nitrogen--;  
Line 17, after "required for" insert --quenched  
and--;  
Line 32, after "FIG. 1" change "and" to --to--;  
Line 52, change "restrict" to --retard--;  
Line 53, change "content" to --addition--;

Column 8, Line 5, change "reduction" to --reductions--;  
Line 6, change "a constant reduction" to  
--the constant reductions--;  
Line 15 to after "respectively." delete the following  
Line 19 entire sentence and substitute therefore  
--Table 3 also shows the lower limit  
reduction values for dynamic recrystalliza-  
tion determined from the values of  
 $N\sqrt{R_o/H}$  in Table 2, the reduction  
temperatures and FIG.1.--

Column 9, Line 25, change "waiting time" to --further  
Line 25, waiting--;  
Line 41, after "seconds" insert --occurs--;  
change "a flat slab" to --flat slabs--;

Column 11, Line 16, after "Table 1" insert --was--;  
Line 16, change "flat slabs" to --a flat slab--;  
Line 27, change "second" to --first--;  
Line 28, change "first" to --second--;  
Line 53, change "properites that" to --properties as  
compared with--;

UNITED STATES PATENT OFFICE page 3 of 3  
CERTIFICATE OF CORRECTION

Patent No. 3,918,999 Dated November 11, 1975

Inventor(s) Hiroshi Sekine; Tadakatsu Maruyama; Katsutoshi Yamada

It is certified that error appears in the above-identified patent and that said Letters Patent are hereby corrected as shown below:

Column 13, Table 9, Schedule 9, Line  $N\sqrt{R_o/H}$  (rpm),  
under "Eighth Reduction" change "72" to --73--;

Column 15, Table 12-continued, below the heading "Low Temperature Rolling Conditions" change "schedules 9 and 10" to read --schedules 10 and 11--.

Signed and Sealed this

Twenty-fourth Day of August 1976

[SEAL]

Attest:

**RUTH C. MASON**  
Attesting Officer

**C. MARSHALL DANN**  
Commissioner of Patents and Trademarks